

# UNITED STATES PATENT OFFICE.

ERNST J. WATZL, OF CLEVELAND, OHIO, ASSIGNOR TO NATIONAL CARBON COMPANY,  
OF CLEVELAND, OHIO, A CORPORATION OF NEW JERSEY.

## ARC-LAMP ELECTRODE.

1,161,173.

Specification of Letters Patent. Patented Nov. 23, 1915.

No Drawing.

Application filed April 14, 1913. Serial No. 761,056.

To all whom it may concern:

Be it known that I, ERNST J. WATZL, a subject of the Emperor of Austria-Hungary, residing at Cleveland, in the county 5 of Cuyahoga and State of Ohio, have invented a certain new and useful Improvement in Arc-Lamp Electrodes, of which the following is a full, clear, and exact description.

10 My invention relates to electric arc electrodes adapted to produce flaming or luminous arcs.

In constructing flaming arc electrodes, certain materials are added to support the 15 arc for enabling a long arc to be drawn while other materials are added for the purpose of increasing the candle power and improving the color. Tungstic oxid belongs in the first class mentioned, and is therefore 20 used more or less in flaming electrodes as an arc supporter. Titanium materials and rare earth compounds belong in the second class, both furnishing a high candle power of an intense whiteness.

25 It is the object of my invention to combine rare earth oxids, titanium oxid and tungstic oxid in correct proportions to form a chemical compound and obtain all the advantages of each individual constituent and 30 also further advantages due to their chemical union.

I have found that oxids of the rare earths, titanium and tungsten, will combine in molecular proportions to form a chemical 35 compound. These, as far as I have been able to find out in my experiments combine in a great many different proportions, but always in the ratio of their molecular weights, *i. e.*, the chemical compound has 40 the composition



where *m*, *n* and *p* represent the variable proportions of the oxids, and RE represents the 45 rare earths, which substantially consist of 52% cerium oxid, 45% of lanthanum and didymium and 3% yttrium, ytterbium and thorium.

Tungstic oxid is expensive and, therefore, 50 I prefer to form the compound with as low a content of this substance as efficiency will

permit. I have found a compound having the formula



55

makes an excellent ingredient for arc lamp electrodes. To form the compound, I mix together the three oxids in substantially this proportion, and heat them to a very high temperature by means of an electric arc furnace. This temperature is probably 2500 degrees or more. Under the heat of the arc, the materials fuse and unite as a definite chemical composition. That the resulting material is a chemical compound is evi- 60 denced by the fact that the density is over 30% greater than would be the density of the same materials in a mechanical mixture; that the product is of uniform structure under the microscope; and that it crystallizes 65 in regular monoclinic form. After the material is fused and cooled, it is easily crushed and can be mixed with carbon, calcium fluorid, and other well known constituents of flaming electrodes and formed into the 70 75 desired shape.

If the three oxids are mechanically mixed together and included in a lamp electrode, only a small percentage would unite to form the chemical compound, as tungstic oxid and 80 titanium oxid fuse at a much lower temperature than the rare earth oxids. When unrestricted by inclosing walls, the oxids of titanium and tungsten will vaporize first and will not unite with the rare earth oxids, 85 hence, to obtain the full advantage of the chemical compound, it is necessary to form it before it is put in the lamp electrode. I have also found that, when the three oxids are mechanically mixed together, the arc 90 formed between the electrodes is somewhat unsteady due to flickering. When the material is placed in the lamp electrode in the form of a chemical compound the unsteadiness is much reduced. The chemical com- 95 pound is of greater density than the mechanical mixture and therefore more of it can be included in a lamp electrode. Also the denser the material, the more efficient it is as a constituent of a lamp electrode 100 and for this reason the materials when united as a chemical compound produce a

more efficient light than when mechanically mixed together.

While I have explained the use of the oxids in forming my improved compound, it must be understood that other forms such as the carbonates may be used. On account of the smaller cost of rare earth carbonates as compared to rear earth oxids, I prefer to use the former instead of the latter.

- 10 My improved compound can be used in various proportions with other materials to form the electrode, but I have found that excellent results are obtained by forming about 16% of the electrode of the compound.
- 15 Having described my invention, what I claim is:

1. An arc lamp electrode containing the oxids of titanium, tungsten and the rare earths chemically united.

2. An arc lamp electrode having as one of its constituents a material consisting of compounds of titanium, tungsten and the rare earths chemically united.

3. An are lamp electrode containing the fused oxids of titanium, tungsten, and the rare earths in molecular proportions.

In testimony whereof, I hereunto affix my signature.

ERNST J. WATZL.

Witnesses:

IRV J. ADAMS,  
D. BREWER.